

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## METAL FILAMENT.

1,026,384.

Specification of Letters Patent.

Patented May 14, 1912.

No Drawing.

Application filed September 23, 1908. Serial No. 454,446.

*To all whom it may concern:*

Be it known that I, WILLIAM D. COOLIDGE, a citizen of the United States, residing at Schenectady, in the county of Schenectady and State of New York, have invented certain new and useful Improvements in Metal Filaments, of which the following is a specification.

I have developed a process for making filaments of refractory material such as tungsten, molybdenum, titanium, boron, and other refractory powders of various kinds, by utilizing as a binding material for the powder, a ductile alloy having such characteristics that it can be impregnated with the powder and then extruded through a die to shape the mixture into wires. After wires have thus been formed consisting of a conglomerate mixture of metal binder and refractory powder, I heat them in suitable manner to drive out the binder and to shrink and sinter the refractory residue into firm coherent conductors suitable for use as lamp filaments.

According to my present invention, I add to a conglomerate mixture of the type above mentioned, a diluting compound of such a nature that on heating it will react with one of the metallic components of the mixture to form a porous material and a pure metal. The latter serves as a binder for the other components until driven out at higher heat treatments, while the porous material serves to soak up the liquid constituents during the early stages of the heat treatment, thereby preventing the formation of globules of fused metal along the wire under treatment and otherwise assisting in the production of a uniform refractory conductor or filament.

The components of this diluting compound are eventually driven from the filament with the result that the finished filament is of considerably less diameter than the original wire. This feature is of importance as tending to cheapen production and as rendering easy the manufacture of lamp filaments of exceedingly small cross-section.

Although my process is a general one, I will proceed by describing one embodiment employed by me with success.

Powdered tungsten and powdered cupric oxid are rubbed into a warm and plastic amalgam consisting of 44 parts cadmium to 44 parts mercury to 12 parts bismuth. The

mixture of tungsten and oxid is added to 55 the amalgam to the extent of 35 per cent. Of this mixture the relative proportions between tungsten and oxid may vary through wide limits, as from a very small percentage of oxid to 75 parts oxid and 25 parts 60 tungsten, according to the amount of shrinkage desired, the amount of metal binder produced from the compound, and the amount of porous material for soaking liquid constituents of the initial binder found 65 desirable in any particular case. The conglomerate mass thus produced consists of the cadmium-bismuth amalgam acting as a binder and the powdered tungsten and cupric oxid held in place by the binder. 70 This mixture is next squirted warm through a diamond die and comes out as a silver white ductile wire. This wire is cut into suitable lengths and then baked in an evacuated glass tube heated with a gas flame to a 75 temperature at which the mercury and possibly some of the cadmium distil from the wire. This heat treatment also produces another important change in the wire, namely, that of causing chemical reaction 80 between the cadmium of the amalgam and the cupric oxid added as a diluent, thereby producing metallic copper and cadmium oxid. This reaction goes on very easily and smoothly and the temperature need not 85 greatly exceed 300 degrees C.

When the filaments come from the baking operation they consist of tungsten powder and cadmium oxid held together by a binder of bismuth, copper, and possibly some cadmium. The amount of the latter component depends, of course, on the proportion of cupric oxid added to the mixture, for if a small quantity only is added then more cadmium will remain behind unoxidized. In 90 the next step, the filaments are heated in a vacuum to a higher temperature, to produce vaporization of the cadmium and of the bismuth, and finally, vaporization of the copper and direct distillation of the cadmium 100 oxid. Inasmuch as the cadmium oxid comes off last it is present when the cadmium and bismuth change over from the solid to the liquid state and can therefore operate to soak up the liquid metal and keep it from 105 running together into globules during that interval of time before the temperature is high enough to produce complete vaporiza-

zation. After the binding material and the diluent are all out of the filament, the temperature may be still further increased to sinter and shrink the tungsten and render it more stable and otherwise better suited for use in an incandescent lamp. This heat treatment may be effected by current passed directly through the filament or in any other suitable manner. Inasmuch as the process is operative with high percentage of diluent, it is altogether possible to produce a finished tungsten filament having a diameter much less than that of the die through which the original plastic mass was squirted.

According to the procedure above described, the removal of the vaporizable components is effected in a vacuum. If desired, an atmosphere of hydrogen may be used during this treatment in which case the 15 cadmium and bismuth come out as before but the cadmium oxid is reduced by the hydrogen and leaves the filament prior to vaporization of the copper.

As a typical embodiment of my invention, I have disclosed the use of cupric oxid. 20 This is a good material for this purpose as it can be obtained in fine and pure condition by simply oxidizing in air the very fine copper carbonates now on the market as 25 pigments. Furthermore, the cupric oxid will react with the cadmium within the comparatively small temperature range between the removal of the mercury and the removal of the cadmium by baking. And in addition, the copper liberated from the oxid does 30 not in any way contaminate the tungsten or impair its refractory qualities. I do not, however, wish to be limited as to the scope 35 of this process, except by the appended 40 claims.

What I claim as new and desire to secure by Letters Patent of the United States, is,

1. The method which consists in producing a ductile mixture containing a metallic binder, a finely divided refractory material, 45 and a diluent capable of combining with one component of the binder, forming a body of desired shape therefrom, effecting chemical reaction between said diluent and said 50 binder and then removing from said mixture all components except said highly refractory material.

2. The method which consists in forming wires containing a metallic binder, a highly 55 refractory powder and a chemical compound, heating to cause reaction between said compound and one component of said binder, and subsequently heating to a higher temperature to drive from the wire all components except said highly refractory material.

3. The method which consists in producing a wire containing a cadmium alloy, tungsten and cupric oxid, heating to effect 60 oxidation of at least part of said cadmium,

and subsequently heating to a higher temperature to successively drive out all easily vaporizable components.

4. The method which consists in forming a wire containing a metallic binder, a finely divided refractory material and a chemical compound capable of reacting with one component of said binder to produce a relatively stable material, heating to effect this chemical reaction and then heating to higher temperatures to remove from the wire all components except said highly refractory material.

5. A ductile wire consisting of a refractory powder, a chemical compound and a metallic binder, said compound being such that it will react chemically with one component of said binder to form a relatively stable material.

6. A wire consisting of a cadmium alloy, 85 a refractory powder and a compound capable of reacting with cadmium to produce a porous and relatively stable material.

7. A wire consisting of a cadmium amalgam, cupric oxid, and a finely divided refractory material.

8. A wire containing cadmium, bismuth, mercury, tungsten and cupric oxid.

9. The method which consists in heating a wire containing refractory material, metallic binder, and suitable metal compound to cause chemical reaction between said compound and at least a portion of said binder and eliminate all substances except said refractory material and produce a filamentary body containing only said refractory material and to produce by said reaction a relatively stable porous compound of an element of said binder.

10. The method which consists in forming 105 a body of desired shape containing refractory material, metallic binder, and compound of metal having a higher point of fusion than said binder, heating to cause chemical reaction between said compound and said 110 binder and by said reaction producing a relatively stable porous compound of an element of said binder and liberation of said higher melting metal, and to eliminate all 115 substances except said refractory material.

11. The process of treating a filamentary body containing refractory material and binding material plastic at relatively low temperature and additional material which consists in heating said body to effect removal of said binding material and to cause the additional material to become effective 120 as a coherent metallic binder of fusion temperature approximating the temperature at which heat tends to consolidate the refractory material, and then heating to a higher 125 temperature to remove said additional material and to produce a coherent body containing only said refractory material.

12. A wire containing refractory material, 130

low melting metal binder, and compound of higher melting metal, said compound being capable of reacting with said binder with resulting liberation of said higher melting metal.

13. An unfinished filamentary body comprising refractory material, low-melting metal binder, and higher melting metal capable of remaining in said body at a temperature under which said refractory material tends to consolidate.

14. The process which consists in forming a filamentary body containing material initially effective as binder and metallic compound and treating such body to cause the liberation from such compound of metal which acts as binder for maintaining the filamentary body in a coherent condition until it begins to possess coherence independently of any binder and convert it into a filament consisting wholly of refractory material.

15. The process which consists in forming a mixture containing refractory material and material initially effective as binder and other material, shaping said mixture as desired, and treating the shaped body to cause such other material in the mixture to become an effective binder to maintain the body in a coherent condition until the refractory material itself begins to cohere and

convert it into one consisting wholly of refractory material.

16. The method of converting a filamentary body containing material initially effective as binder and other material into a coherent refractory body which consists in first heating to remove the material initially effective as binder and to cause such other material to become an effective binder for maintaining the filamentary body in a coherent condition for subsequent treatment and then heating to a higher temperature to eliminate everything except a refractory residue from the filament and consolidate such residue.

17. A mixture for the production of refractory bodies comprising material which is initially effective as binder to allow shaping of the mixture and other material which becomes an effective binder during the process of converting the shaped body into a coherent refractory one and serves to maintain the body in a coherent condition during such process.

In witness whereof, I have hereunto set my hand this 21st day of September, 1908.

WILLIAM D. COOLIDGE.

Witnesses:

BENJAMIN B. HULL,  
MARGARET E. WOOLLEY.